

(No Model.)

C. M. LUNGREN.  
INCANDESCENT GAS LIGHT.

No. 439,882.

Patented Nov. 4, 1890.



Fig. 1.



Fig. 1A.



Fig. 2.

Fig. 4.



Fig. 4A



Fig. 2A

Fig. 3.



Fig. 3A. Inventor

Charles M. Lungren

By Attorney

Frank MacArthur

Witnesses

Ira R. Steward,  
Curtis Lammond

# UNITED STATES PATENT OFFICE.

CHARLES M. LUNGREN, OF BROOKLYN, NEW YORK.

## INCANDESCENT GAS-LIGHT.

SPECIFICATION forming part of Letters Patent No. 439,882, dated November 4, 1890.

Application filed April 9, 1889. Serial No. 306,498. (No model.)

*To all whom it may concern:*

Be it known that I, CHARLES M. LUNGREN, a citizen of the United States, residing at Brooklyn, in the county of Kings, in the State 5 of New York, have invented certain new and useful Improvements in Incandescent Gas-Lights, of which the following is a description.

My invention relates to an improved method 10 of making filamentary bodies composed of the refractory earths or metallic oxides to be used in incandescent gas-lighting; and it consists in weaving or otherwise interlacing threads or wires of the metallic oxides or refractory earths into the form of an open mesh 15 or net-work, the mesh or net-work being arranged in any suitable shape adapted to the flame, such as a cone or tube.

As heretofore practiced, the method has 20 been to wind the threads comprising the structure upon a mandrel of the desired shape and to press them together at the points of crossing. In making a cone, for instance, all or part of the threads running 25 lengthwise of the conical mandrel are wound. Then the coil is wound over these, and where the two cross they are pressed together. When the threads are fine, there is great danger in this method of construction of cutting them 30 in two when the pressure is sufficient to make them adhere. A more important objection to this method of construction is, however, the rigidity of the resulting structure, which prevents the parts expanding and contracting 35 freely under the changes of temperature to which the structure is designed to be subjected. To obviate these objections I weave or otherwise interlace the threads composing the structure, which leaves all the parts free 40 to move with regard to each other, while at the same time they are held in place and the form of the structure as a whole is preserved. In the drawings I have shown four different forms of such interlacing as applied to a conical structure.

In Figures 1 and 1<sup>A</sup> the thread of refractory earth is shown disposed in a series of loops caught the one to the other, the arrangement being that produced by knitting. In Figs. 2 45 and 2<sup>A</sup> the threads are made to pass over and under each other in opposite diagonal direc-

tions, the construction being that produced by a braiding-machine. In Figs. 3 and 3<sup>A</sup> is shown a sample of weaving proper. By appropriate mechanism half of the vertical 55 threads are alternately carried above and below the horizontal thread, the operation being precisely that of a loom. In Figs. 4 and 4<sup>A</sup> is shown a form of interweaving produced by twisting alternate verticals about each 60 other. This is produced by means of a special machine, which will form the subject of a separate application.

To handle a thread of the refractory earths in any of these ways requires that it should 65 be very plastic and remain so for a considerable length of time and that it should have considerable tensile strength. These qualities may be obtained by the use of a variety of binding materials. By the addition of 70 glycerine to glue or allied binding materials the hardening of the glue is prevented and threads may be produced which will remain sufficiently plastic for the purpose. The class of binders soluble in the oils or ethers may 75 also be used—such as rubber cement (pure rubber dissolved in naphtha) or burned linseed-oil, (printers' varnish.) In preparing such threads I mix the refractory earth—such as magnesia—with the binder and work the 80 two together until a plastic mass of the requisite consistency is obtained. The plastic mass is then put in a press and a thread or wire of the desired size expressed through the die. These threads or wires may then be wound on 85 a reel or bobbin, and are preferably coated with plumbago on the way to prevent adherence of adjacent threads. This result can be readily accomplished by passing the thread through a guide supplied with plumbago. When the 90 thread is desired for use, it is cut up into any desired lengths and used in the weaving, braiding, or knitting machines in the same manner as thread or yarn. After the structures are complete they are burned in a furnace at a high temperature to remove the combustible binder and to harden the refractory earth. They are then ready for use.

I claim—

1. The herein-described method of making 100 incandescents of the refractory metallic oxides or earths, which consists in expressing

threads or wires from a plastic mass and then weaving or otherwise interlacing these threads or wires into structures of the desired form.

5 2. The herein-described method of making incandescent filamentary bodies composed of the refractory earths or metallic oxides, which consists in weaving or otherwise interlacing threads or wires of such material into

the form of an open mesh or net-work of suitable shape, substantially as described.

In testimony whereof I have hereunto set my hand this 30th day of March, A. D: 1889.

CHARLES M. LUNGREN.

Witnesses:

THORNE S. WALLING,  
FREDERIC CARRAGAN.